

B.R. Cotton's  
Improved Dresser Roll.

71991

PATENTED  
DEC 10 1867

B.



A.



B.R. Cotton  
by his Atys  
Witnesses  
{ C. Warren Brown, G. W. H. Elston & Gould  
L. H. Latimer

# United States Patent Office.

BENJAMIN R. COTTON, OF LEWISTON, MAINE.

*Letters Patent No. 71,991, dated December 10, 1867.*

## IMPROVEMENT IN ROLLERS FOR DRESSING.

The Schedule referred to in these Letters Patent and making part of the same.

TO ALL WHOM IT MAY CONCERN:

Be it known that I, BENJAMIN R. COTTON, of Lewiston, Androscoggin county, State of Maine, have invented an Improved Dresser-Roll; and I do hereby declare that the following, taken in connection with the drawings which accompany and form part of this specification, is a description of my invention sufficient to enable those skilled in the art to practise it.

United States Letters Patent, No. 64,078, were granted to me, April 23, 1867, for an improved dresser-roll, the improvement consisting in surfacing or covering the roll with a composition of lead and tin, or an analogous alloy or metal, which resists the action of the size, does not become creased, and has and preserves an even surface. Said invention is described as particularly applicable to metal rolls, the surfacing-metal being united to the roller-metal by "soldering," by depositing with a battery, or by casting. But the invention is also applicable to other rolls, the improvement consisting rather in making a dresser-roll with such a surface than in surfacing particular rolls. My present invention, however, relates particularly to covering stone rolls with such metal or composition having particular reference to metal-surfacing old soapstone dresser-rolls.

The invention consists primarily in surfacing a stone roll with the metal by first covering the stone roll with a metal frame, and then casting, soldering, or depositing upon this frame the metal which is to constitute the surface of the dresser-roll, such surface being subsequently turned down to cylindrical shape.

The drawings represent a roll embodying this improvement.

A shows the roll in elevation, with a part of the outer surface broken away to show the frame and stone surface beneath.

B shows the roll in cross-section.

a denotes the stone roll, around the cylindrical surface of which, from end to end, I wind a copper, brass, galvanized iron, or other suitable wire, b, and upon this I cast, solder, or deposit the surface-metal c. The mode of surfacing which I have particularly used has been to lay bars of solder lengthwise upon the wire, and to melt the same over the wire with a soldering-iron, but other methods may of course be used, and may be found to be preferable. Having effected the covering of the wire, the surface-metal is then turned down to give a true cylindrical shape to the roll. Instead of using the wire, a tin, sheet-iron, or other metal tube may be drawn over the stone roll, or a strip of sheet metal may be wound thereupon and the surface-metal laid upon and cemented thereto, and metal rolls may be similarly covered by laying a frame or coil of metal around each as a base to which to unite the surface-metal or alloy.

I claim as an improved dresser-roll, a stone roll covered with the surfacing-metal or metal composition, substantially as set forth.

I also claim the method of surfacing a roll, by placing around or over a central roll a metal frame as a base upon which to cement the surface-metal, and the surfacing such frame, substantially as set forth.

BENJAMIN R. COTTON.

Witnesses:

T. A. D. FESSENDEN,

JOHN B. COTTON.